

Nov. 20, 1923

1,474,800

R. C. STIEFEL

METHOD OF MAKING SEAMLESS TUBES

Filed June 16, 1920



INVENTOR

Ralph C. Stiebel  
By Hunter & Brown  
Attorneys

Patented Nov. 20, 1923.

1,474,800

# UNITED STATES PATENT OFFICE.

RALPH C. STIEFEL, OF ELLWOOD CITY, PENNSYLVANIA.

## METHOD OF MAKING SEAMLESS TUBES.

Application filed June 16, 1920. Serial No. 389,348.

*To all whom it may concern:*

Be it known that I, RALPH C. STIEFEL, a citizen of the United States, and a resident of Ellwood City, in the county of Allegheny and State of Pennsylvania, have invented a new and useful Improvement in Methods of Making Seamless Tubes, of which the following is a specification.

The invention is a method of making 10 seamless tubes which has the hereinafter enumerated advantages over the methods heretofore employed.

According to the most generally followed present method of making seamless tubes, 15 the solid billet is pierced to a rather thin wall, the hollow billet is then given several passes through a grooved mill over a stationary plug, known as a plug-mill, and is therein reduced to a blank having a wall 20 thickness and diameter substantially that of the desired finished tube, and said tube is then cross rolled or "reeled" over a mandrel to smooth out any interior grooves or 25 ridges and exterior roughness produced in the plug-mill, true the gage and round the tube.

In the reeling step no material reduction 30 of wall thickness or change in diameter is made, due to the character of the rolls employed, and their action. Consequently the entire reduction in wall thickness must be 35 made in the piercing and plug-rolling operations, and since in the plug-rolling operation the blank is brought down to the desired finished wall thickness it cools quite rapidly so that there is a limit to the number of 40 passes which can be given in the plug-mill. This has necessitated piercing the billet to as thin a wall as is practical, in order that it can be reduced to the finished wall thickness in a limited number of passes which 45 can be given in the plug-mill before the blank cools excessively. Piercing the solid billet to a thin wall obviously produces a heavy strain on the steel, and is liable to tear it, but in any event to aggravate any 50 seams or defects existing in the solid steel billet.

Furthermore, while in the piercing operation 55 the diameter of the blank can be increased to a limited extent beyond that of the solid billet, such slight increase in diameter is offset in the plug-rolling operation where the effect is to reduce the diameter of the blank while thinning and elongating it, and in the reeling operation, as already

stated, there is no material increase in diameter. Consequently in all cases the solid billet must be of substantially the same diameter as the finished tube, as a result of 60 which the method does not lend itself well to the production of tubes of large diameter, and for any given size of tubes leads to a large percentage of rejections due to defects in the metal, as will hereinafter appear.

My improved method, generally stated, comprises the steps of piercing the solid billet, then plug-rolling the hollow blank, and then subjecting the blank to the action 70 of cross rolls of the kind known as expanding rolls, which latter step still further and very substantially reduces the thickness of the walls and increases the diameter of the tube, while at the same time eliminating or 75 reducing any scores or irregularities and smoothing the tube both internally and externally. Because in this cross-rolling operation the wall thickness is substantially reduced, it is not necessary to bring the blank 80 to the expanding rolls with its walls reduced to substantially the finished gage. Consequently the billet can be pierced with a thicker 85 wall, thus imposing less strain on the steel, and also giving a blank which is softer and at a better rolling heat than with the old thin walled pierced billets, and which therefore can be more quickly and easily reduced in the plug-mill and with a better effect on the metal. Furthermore, since in the plug- 90 rolling the blank is not reduced to the desired finished wall thickness it also goes to the cross rolls at a higher temperature than in the existing method, and can therefore be effectively and easily reduced to the 95 final desired gage. Since in the expanding rolls the tube is substantially increased in diameter this method, for a given size of tube, permits of the use of a billet of less 100 diameter than is possible under the old method. This has important advantages as will hereinafter appear.

In the accompanying drawings Fig. 1 illustrates diagrammatically the piercing operation; Fig. 2 similarly illustrates the 105 plug-rolling operation; and Fig. 3 similarly illustrates the cross-rolling and expanding operation.

The piercing mill may be of any desired type, that shown in Fig. 1 comprising a 110 pair of barrel shaped rolls 5 provided with the usual pass which first converges and

then diverges and having lying in the exit side of the pass the usual piercing plug or point 6. The solid billet 7 is here pierced and somewhat expanded, forming a hollow blank 8 which differs from the usual pierced blank only in that it need not be reduced to as thin a wall as has heretofore been the practice.

The pierced blank then goes to the plug-rolling mill which may be of any desired form, that shown in Fig. 2 comprising a pair of grooved rolls 9 provided with a plurality of passes in which lie suitable plugs 10 held by bars 11. In this mill the hollow blank is given one or more passes, as necessary, preferably a plurality of passes, and is reduced therein to a wall thickness substantially greater than that of the desired finished tube. This mill will be so organized that the several passes therethrough follow each other in quick succession, to secure the necessary reduction with as little loss of heat as possible. In this mill the blank is not only elongated and the walls thinned, but because of the relative high temperature of the blank during this operation any seams or defects inherent in the steel and aggravated in the piercing operation, or produced by the piercing operation, are closed and welded to a greater extent than with the thinner and colder blanks which are plug-rolled under the old process.

The blank 12 then goes to the cross-rolling or expanding mill, shown in Fig. 3, comprising the conical rolls 13 (or their equivalent) which provide a pass which slightly converges at the entrance side and materially diverges on the delivery side and having lying in such pass on the delivery side the conical plug 14 held by the bar 15. In this mill the blank is very substantially expanded, thus producing a substantial reduction in wall thickness and an increase in diameter, and is therein reduced to the desired finished wall thickness and diameter. At the same time the cross-rolling under the external rolls and internal mandrel eliminates any interior grooves or scores and external roughness produced in the plug rolling operation, thus smoothing the tube inside and outside, and also equalizes and trues the wall thickness and rounds the tube, so that the tube delivered is commercially salable as a hot finished tube.

The several mills described will be so arranged that the blank can be quickly and conveniently transferred from one to the other, in order that the heat may be conserved. The entire rolling operation described can be readily performed at the initial heat of the billet, but if necessary the blank can be reheated between operations.

From the cross-rolling or expanding mill the tube is preferably passed through the well-known sizing rolls to reduce it to exactly the desired diameter. Where tubes of

superior finish are desired, the hot finished tube produced by the above described operations will be cold drawn in the usual way.

The advantages of the foregoing described method will be readily appreciated by those skilled in the art. Since in the cross-rolling step the blank is very substantially increased in diameter, it is possible for any given sized tube to start with a solid billet of less diameter than the old method. This is not only a great advantage in the manufacture of large diameter tubes but for any given size of tubes the billet will be sounder and will have less seams or defects, or at least of less depth, than the corresponding billet which is necessary under the old method, because in steel mill practice the billets are produced from standard sizes of ingots, and manifestly the smaller the diameter of the billet the greater the amount of rolling necessary to bring it to size and consequently the more work expended on the steel and the better the quality of the steel. Any seams or other defects existing in the ingot are less, and are of relatively less depth in a small sized billet than in a large sized billet rolled from the same ingot. It is also of great advantage to pierce with thick walls as thereby the metal is tortured less and hence the defects in the steel are aggravated to a lesser extent than under the old method, and tearing and seaming of the metal is also largely avoided.

The thick walled hollow billet has the further obvious advantage that it will hold its heat more effectively than a thin walled hollow billet, and consequently it is softer and at a better rolling temperature for plug-rolling so that the latter step can be more easily and quickly carried out and in addition any defects in the metal or seams which may have been produced in the piercing operation are, by the compressing action on the metal while confined between the rolls or grooves on the outside and the plug or mandrel on the inside, closed and welded more effectively and to a greater extent than under the old method. The net result is that the percentage of rejections due to defects or seams in the tubes is much less than under the old method. Furthermore, because the tube is not reduced to the desired final wall thickness and diameter in the plug-mill, this operation is less exacting than under the old method, and in addition leaves the tube at a better temperature for the subsequent cross-rolling step. The cross-rolling thus becomes easier and in addition eccentricity is reduced because of the greater softness of the thicker portion of the tube wall.

I claim:

1. The method of making seamless tubes which consists in rolling a relatively thick walled hollow billet in a plug-mill to a tube of less diameter and greater wall thickness

than the desired finished tube and simultaneously closing or welding seams and defects in the metal, and then cross-rolling and expanding the blank over a mandrel plug in 5 a manner to increase its diameter and reduce its wall thickness to the desired diameter and wall thickness, and simultaneously smoothing the tube inside and outside, rounding it, and truing and equalizing its 10 walls.

2. The method of making seamless tubes which consists in piercing a solid billet to form a relatively thick walled blank, then rolling said blank in a plug-mill and thereby elongating and thinning its walls and

producing a blank of less diameter and greater wall thickness than the desired tube, and then cross-rolling and expanding said blank over a mandrel plug in a manner to reduce its wall thickness and increase its diameter to the desired wall thickness and diameter, and simultaneously smoothing the tube internally and externally, rounding it, and truing and equalizing its walls. 20

In testimony whereof, I have hereunto set 25 my hand.

RALPH C. STIEFEL.

Witness:

HOWARD T. SNIVELY.